

## 1

3,579,342

### LEUCO TRIARYLMETHANE/HEXAARYLBIIMIDAZOLE COLOR FORMING SYSTEM CONTAINING A DEACTIVATOR

Peter S. Strliko, Wilmington, Del., assignor to E. I. du Pont de Nemours and Company, Wilmington, Del.  
No Drawing. Filed June 27, 1968, Ser. No. 740,476  
Int. Cl. G03c 1/72

U.S. Cl. 96—90

14 Claims

#### ABSTRACT OF THE DISCLOSURE

A photoimagable and photodeactivatable composition of  
(A) A salt of a leuco triarylmethane and a salt-forming acid;

(B) A hexaarylbiimidazole which absorbs principally in the ultraviolet region and is a photooxidant for the salt of the leuco triarylmethane present in an amount of from about 1 to 2 moles per mole of said salt of the leuco triarylmethane;

(C) 1,6-pyrenequinone or 1,8-pyrenequinone or both, present in an amount of from about .04 to .4 mole per mole of hexaarylbiimidazole;

(D) A visible light-absorbing carbonyl compound selected from 9,10-phenanthrenequinone, perinaphthenone, or 4-methoxy-1,2-naphthoquinone; present in an amount of from about .05 to 2 moles per mole of hexaarylbiimidazole; and

(E) An ether containing at least one oxymethylene group wherein the methylene bears at least one hydrogen; present in an amount providing from about 50 to 500 oxymethylene groups per mole of the combined quinone components (C) and (D).

#### BACKGROUND OF THE INVENTION

##### (1) Field of the invention

This invention relates to photosensitive compositions. More particularly it is directed to an admixture of a photoactivatable color-forming system comprising a salt of a leuco triarylmethane and a hexaarylbiimidazole, and a system for photodeactivating the color-forming system comprising a mixture of selected quinones and an aliphatic ether.

##### (2) Description of the prior art

British Pat. 1,047,569 discloses the color-forming system employed in the present invention and discloses that the leuco triarylmethane/hexaarylbiimidazole combination forms color on exposure to ultraviolet light. British Pat. 1,057,785 discloses that the leuco triarylmethane/hexaarylbiimidazole system can be deactivated against color formation with light of a second wavelength, by incorporating therewith a light activatable oxidation-reduction system which on radiation with the light of a second wavelength produces a reducing agent which reacts with the photolyzed hexaarylbiimidazole, thus preventing color formation.

One photoactivatable oxidation-reduction system disclosed by British Pat. 1,057,785 involves a visible-light activatable quinone in combination with a polyether bearing an extractable hydrogen. Irradiation of the British Pat. 1,057,785 system with ultraviolet light produces color corresponding to the dye form of the leuco triarylmethane; while irradiation with visible light deactivates the color-forming components against color formation. The deactivation of the color-forming components is attributable to in situ hydroquinone formation from the quinone employed, which then reacts with the photolyzed hexaarylbiimidazole.

Since the hexaarylbiimidazoles can absorb at wave-

## 2

lengths as high as 430 m $\mu$ , which are the violet wavelengths, the compositions of British Pat. 1,057,785, tend to form some color when irradiated with the deactivating visible light radiation. Since color formation is ordinarily undesirable during the deactivating step, it is suppressed by controlling the deactivating conditions. A filter can be employed to screen activating radiation from the color-forming components; a monochromatic light can be employed that only the deactivating components can absorb; or a light source can be employed which emits principally in the photodeactivation region with substantially no light emitted in the region of hexaarylbiimidazole absorption.

However, in some applications it is desirable to eliminate the need for deactivating under controlled conditions.

5 This can be accomplished by providing for rapid photodeactivation, i.e., by employing deactivation components which react to deactivate so rapidly that the competing color-formation reaction cannot get underway. By employing such components, color formation can be prevented from occurring upon exposure of the system to light such as sunlight, roomlight or daylight, which contains intense violet wavelengths.

U.S. Pat. 3,390,994, issued July 2, 1968, describes a rapidly photodeactivatable system for use with the leuco 25 triarylmethane/hexaarylbiimidazole color-forming components which employs either pyrenequinone or phenanthrenequinone as the oxidant member of the deactivating system and an alkyl nitrilotriacetate or alkyl nitrilotripropionate as the reductant member. Although this system possesses rapid deactivation properties, it tends to 30 form color rather slowly and tends to be limited in its maximum color attainment. Moreover, it is sensitive to human handling. When coatings of it are touched prior to irradiation for color formation, these touched areas are 35 not imaged and appear as uncolored fingerprint areas after the coating is subsequently irradiated with color-forming irradiation.

It is an object of this invention to provide photosensitive compositions which form color rapidly, which attain 40 maximum color, and which are not sensitive to "fingerprinting." These and other objects of the invention will become apparent hereinbelow.

#### SUMMARY OF THE INVENTION

45 The photosensitive compositions of this invention comprise an intimate admixture of

(A) A salt of a leuco triarylmethane and a salt-forming acid;

(B) A hexaarylbiimidazole which absorbs principally 50 in the ultraviolet region and is a photooxidant for the salt of the leuco triarylmethane present in an amount of from about 1 to 2 moles per mole of said salt of the leuco triarylmethane;

(C) 1,6-pyrenequinone or 1,8-pyrenequinone or both, present in an amount of from about 0.04 to 0.4 mole (preferably 0.1 to 0.3 mole) per mole of hexaarylbiimidazole;

(D) A visible light-absorbing carbonyl compound selected from 9,10-phenanthrenequinone, perinaphthenone, or 4-methoxy-1,2-naphthoquinone; present in an amount of from about 0.05 to 2 moles (preferably 0.15 to 0.75 mole) per mole of hexaarylbiimidazole; and

(E) An ether containing at least one oxymethylene group wherein the methylene bears at least one hydrogen; present in an amount providing from about 50 to 500 oxymethylene groups per mole of the combined quinone components (C) and (D).

#### DESCRIPTION OF THE INVENTION

70 In the foregoing definition, components (A) and (B) comprise the color-forming system; while components (C), (D), and (E) comprise the deactivating system.

## 3

The mixture of the quinones of components (C) and (D) with the ether of (E) are critical in achieving the objects of the invention. Use of a single quinone, or any other quinone mixture, or other reductants in place of the ether of (E) fail to result in providing the properties that characterize the invention, particularly, the sunlight, roomlight, or daylight color-formation resistance and the absence of "fingerprinting."

## (1) THE DEACTIVATING SYSTEM

The deactivating components (C), (D) and (E) comprise an oxidation-reduction system which, upon exposure to visible light, react to form a product which deactivates the hexaarylbiiimidazole (B). The oxidant member of the deactivating oxidation-reduction system is a mixture of at least two compounds (one from (C) and one from (D)), which absorb light in the 400 to 500  $\text{m}\mu$  region. Preferably, component (C) is a mixture of both 1,6-pyrenequinone and 1,8-pyrenequinone in molar proportions ranging from 70:30 to 30:70. Preferably, also (D) is 9,10-phenanthrenequinone in an amount of from about 1 to 10 moles per mole of (C) and most preferably in an amount of 1.5 to 2.5 moles per mole of (C); and the mixture of (C) and (D) is 0.1 to 0.2 moles (preferably 0.2 to 1 mole) per mole of (B).

The reductant member of the deactivating oxidation-reduction system is the ether defined in (E). For practicality, it should be substantially non-volatile (boiling at 100° C. and above) and serve to solubilize or plasticize the leuco triarylmethane/hexaarylbiiimidazole/mixed quinone composition so as to provide flexible substantially homogeneous coating compositions and to facilitate both the color-forming and the color-preventing reactions. Suitable reductant members include polyethers containing aliphatic polyether linkages, such as ethyleneoxy or propyleneoxy linkages. These may be represented by the formula



where  $n$  is an integer from 0 to 1;  $m$  is an integer from 1 to 15; R is hydrogen, alkyl, phenyl, alkylphenyl, biphenyl or acyl; R' is hydrogen when  $n$  is zero and is hydrogen, hydroxy or OR when  $n$  is 1. Preferably the alkyl and acyl radicals each contain from 1 to 18 carbon atoms. Most preferably, these reductant members have the formula  $\text{RO}-(\text{CH}_2\text{CH}_2\text{O})_m\text{H}$  where  $m$  is as above and R is phenyl, alkylphenyl or biphenyl.

Representative and preferred classes are the polyethylene glycols such as the commercially available "Carbowaxes"; the analogous polypropylene glycols; and related materials such as phenol-ethylene oxide adducts, for example the ethers and polyethers obtained by reaction of ethylene oxide with o-, m-, p-cresol, o-, m-, and p-phenylphenol and with p-nonylphenol, including such commercially available materials as the "Igepal" alkylphenoxy polyoxyethylene ethanols. Still others are the acetates, propionates, butyrate and other carboxylate esters of the above hydroxy-terminated polyalkyleneoxides and of aliphatic polyols such as ethylene glycol, 1,2-propylene glycol, 1,3-propylene glycol, and glycerol.

Representative materials are additionally described in the examples.

## (2) THE IMAGING SYSTEM

The salt of a leuco triarylmethane is derived from an aminotriarylmethane and a salt-forming acid. Preferably the aminotriarylmethane is one wherein at least two of the aryl groups are phenyl groups having (a) an  $\text{R}_1\text{R}_2\text{N}$ -substituent in the position para to the bond to the methane carbon atom wherein  $\text{R}_1$  and  $\text{R}_2$  are each groups selected from hydrogen,  $\text{C}_1$  to  $\text{C}_{10}$  alkyl, 2-hydroxyethyl, 2-cyanoethyl, benzyl or phenyl, and (b) a group ortho to the bond to the methane carbon atom which is selected from lower alkyl, lower alkoxy, fluorine, chlorine, bromine, or butadienylene which when joined to the phenyl group forms

## 4

a naphthalene ring; and the third aryl group, when different from the first two, is selected from thienyl, furyl, oxazyl, pyridyl, thiazolyl, indolyl, indolinyl, benzoxazolyl, quinolyl, benzothiazolyl, phenyl, naphthyl, or such aforesigned groups substituted with lower alkyl, lower alkoxy, methylenedioxy, fluoro, chloro, bromo, amino, lower alkylamino, lower dialkylamino, lower alkylthio, hydroxy, carboxy, carbonamido, lower carbalkoxy, lower alkylsulfonyl, lower alkylsulfonamido,  $\text{C}_6$  to  $\text{C}_{10}$  arylsulfonamido, nitro or benzylthio. Preferably the third aryl group is the same as the first two.

Particularly preferred aminotriarylmethanes have the following structural formula:



wherein  $\text{R}_3$  and  $\text{R}_4$  are selected from lower alkyl (preferably ethyl) or benzyl, Y and Y' are lower alkyl (preferably methyl) and X is selected from



p-methoxyphenyl, 2-thienyl, phenyl, 1-naphthyl, 2,3-dimethoxy-phenyl, 3,4-methylenedioxyphenyl, or p-benzylthiophenyl. Preferably X is selected from



phenyl, 1-naphthyl, or p-benzylthiophenyl.

These triarylmethanes are employed as salts of strong acids: for example, mineral acids such as hydrochloric, hydrobromic, sulfuric, nitric, phosphoric; organic acids such as acetic, oxalic, p-toluenesulfonic, trichloroacetic acid, trifluoroacetic acid, perfluoroheptanoic acid; and Lewis acid such as zinc chloride, zinc bromide, and ferric chloride; the proportion of acid usually varying from 0.33 mole to 1 mole per amino group. The term "strong acid" as used herein is defined as an acid which forms a salt with an anilino amino group.

Specific examples of the aminotriarylmethanes employed in this invention are:

- bis(4-amino-2-butylphenyl) (p-dimethylaminophenyl) methane
- bis(4-amino-2-chlorophenyl) (p-aminophenyl) methane
- bis(4-amino-3-chlorophenyl) (o-chlorophenyl) methane
- bis(4-amino-3-chlorophenyl) phenylmethane
- bis(4-amino-3,5-diethylphenyl) (o-chlorophenyl) methane
- bis(4-amino-3,5-diethylphenyl) (o-ethoxphenyl) methane
- bis(4-amino-3,5-diethylphenyl) (p-methoxyphenyl) methane
- bis(4-amino-3,5-diethylphenyl) phenylmethane
- bis(4-amino-3-ethylphenyl) (o-chlorophenyl) methane
- bis(p-aminophenyl) (4-amino-m-tolyl) methane
- bis(p-aminophenyl) (o-chlorophenyl) methane
- bis(p-aminophenyl) (p-chlorophenyl) methane
- bis(p-aminophenyl) (2,4-dichlorophenyl) methane
- bis(p-aminophenyl) (2,5-dichlorophenyl) methane
- bis(p-aminophenyl) (2,6-dichlorophenyl) methane
- bis(p-aminophenyl) phenylmethane
- bis(4-amino-o-tolyl) (p-chlorophenyl) methane
- bis(4-amino-o-tolyl) (2,4-dichlorophenyl) methane
- bis(p-anilinophenyl) (4-amino-m-tolyl) methane
- bis(4-benzylamino-2-cyanophenyl) (p-aminophenyl) methane
- bis(p-benzylethylaminophenyl) (p-chlorophenyl) methane
- bis(p-benzylethylaminophenyl) (p-diethylaminophenyl) methane

bis(p-benzylethylaminophenyl) (p-dimethylaminophenyl)  
 methane  
 bis(4-benzylethylamino-o-tolyl) (p-methoxyphenyl)  
 methane  
 bis(p-benzylethylaminophenyl)-phenylmethane  
 bis(4-benzylethylamino-o-tolyl) (o-chlorophenyl)  
 methane  
 bis(4-benzylethylamino-o-tolyl) (p-diethylaminophenyl)  
 methane  
 bis(4-benzylethylamino-o-tolyl) (4-diethylamino-o-tolyl)  
 methane  
 bis(4-benzylethylamino-o-tolyl) (p-dimethylaminophenyl)  
 methane  
 bis[2-chloro-4-(2-diethylaminoethyl)ethylaminophenyl]  
 (o-chlorophenyl) methane  
 bis[p-bis(2-cyanoethyl)aminophenyl]phenylmethane  
 bis[p-(2-cyanoethyl)ethylamino-o-tolyl] (p-di-  
 methylaminophenyl) methane  
 bis[p-(2-cyanoethyl)methylaminophenyl] (p-di-  
 ethylaminophenyl) methane  
 bis(p-dibutylaminophenyl) [p-(2-cyanoethyl)  
 methylaminophenyl] methane  
 bis(p-dibutylaminophenyl) (p-diethylaminophenyl)  
 methane  
 bis(4-diethylamino-2-butoxyphenyl) (p-diethylamino-  
 phenyl) methane  
 bis(4-diethylamino-2-fluorophenyl) o-tolylmethane  
 bis(p-diethylaminophenyl) (p-aminophenyl) methane  
 bis(p-diethylaminophenyl) (4-anilino-1-naphthyl)  
 methane  
 bis(p-diethylaminophenyl) (m-butoxyphenyl) methane  
 bis(p-diethylaminophenyl) (o-chlorophenyl) methane  
 bis(p-diethylaminophenyl) (p-cyanophenyl) methane  
 bis(p-diethylaminophenyl) (2,4-dichlorophenyl) methane  
 bis(p-diethylaminophenyl) (4-diethylamino-1-naphthyl)  
 methane  
 bis(p-diethylaminophenyl) (p-dimethylaminophenyl)  
 methane  
 bis(p-diethylaminophenyl) (4-ethylamino-1-naphthyl)  
 methane  
 bis(p-diethylaminophenyl) 2-naphthylmethane  
 bis(p-diethylaminophenyl) (p-nitrophenyl) methane  
 bis(p-diethylaminophenyl) 2-pyridylmethane  
 bis(p-diethylamino-m-tolyl) (p-diethylaminophenyl)  
 methane  
 bis(4-diethylamino-o-tolyl) (o-chlorophenyl) methane  
 bis(4-diethylamino-o-tolyl) (p-diethylaminophenyl)  
 methane  
 bis(4-diethylamino-o-tolyl) (p-diphenylaminophenyl)  
 methane  
 bis(4-diethylamino-o-tolyl) phenylmethane  
 bis(4-dimethylamino-2-bromophenyl) phenylmethane  
 bis(p-dimethylaminophenyl) (4-anilino-1-naphthyl)  
 methane  
 bis(p-dimethylaminophenyl) (p-butylaminophenyl)  
 methane  
 bis(p-dimethylaminophenyl) (p-sec. butylethylamino-  
 phenyl) methane  
 bis(p-dimethylaminophenyl) (p-chlorophenyl) methane  
 bis(p-dimethylaminophenyl) (p-diethylaminophenyl)  
 methane  
 bis(p-dimethylaminophenyl) (4-dimethylamino-1-  
 naphthyl) methane  
 bis(p-dimethylaminophenyl) (6-dimethylamino-m-tolyl)  
 methane  
 bis(p-dimethylaminophenyl) (4-dimethylamino-o-tolyl)  
 methane  
 bis(p-dimethylaminophenyl) (4-ethylamino-1-naphthyl)  
 methane  
 bis(p-dimethylaminophenyl) (p-hexyloxyphenyl) methane  
 bis(p-dimethylaminophenyl) (p-methoxyphenyl) methane  
 bis(p-dimethylaminophenyl) (5-methyl-2-pyridyl) methane  
 bis(p-dimethylaminophenyl) 2-quinolylmethane  
 bis(p-dimethylaminophenyl) o-tolylmethane

bis(p-dimethylaminophenyl) (1,3,3-trimethyl-2-indolinyl-  
 idenemethyl) methane  
 bis(4-dimethylamino-o-tolyl) (p-aminophenyl) methane  
 bis(4-dimethylamino-o-tolyl) (o-bromophenyl) methane  
 bis(4-dimethylamino-o-tolyl) (o-cyanophenyl) methane  
 bis(4-dimethylamino-o-tolyl) (o-fluorophenyl) methane  
 bis(4-dimethylamino-o-tolyl) 1-naphthylmethane  
 bis(4-dimethylamino-o-tolyl) phenylmethane  
 bis(p-ethylaminophenyl) (o-chlorophenyl) methane  
 bis(4-ethylamino-m-tolyl) (o-methoxyphenyl) methane  
 bis(4-ethylamino-m-tolyl) (p-methoxyphenyl) methane  
 bis(4-ethylamino-m-tolyl) (p-dimethylaminophenyl)  
 methane  
 bis(4-ethylamino-m-tolyl) (p-hydroxyphenyl) methane  
 bis[4-ethyl(2-hydroxyethyl)amino-m-tolyl] (p-diethyl-  
 aminophenyl) methane  
 bis[p-(2-hydroxyethyl)aminophenyl] (o-chlorophenyl)  
 methane  
 bis[p-(bis(2-hydroxyethyl)aminophenyl) (4-diethylamino-  
 o-tolyl) methane  
 bis[p-(2-methoxyethyl)aminophenyl] phenylmethane  
 bis(p-methylaminophenyl) (o-hydroxyphenyl) methane  
 bis(p-propylaminophenyl) (m-bromophenyl) methane  
 tris(4-amino-o-tolyl) methane  
 tris(4-anilino-o-tolyl) methane  
 tris(p-benzylaminophenyl) methane  
 tris[4-bis(2-cyanoethyl)amino-o-tolyl] methane  
 tris[p-(2-cyanoethyl)ethylaminophenyl] methane  
 tris(p-dibutylaminophenyl) methane  
 tris(p-di-n-butylaminophenyl) methane  
 tris(4-diethylamino-2-chlorophenyl) methane  
 tris(p-diethylaminophenyl) methane  
 tris(4-diethylamino-o-tolyl) methane  
 tris(p-diethylamino-o-tolyl) methane  
 tris(p-dihexylamino-o-tolyl) methane  
 tris(4-dimethylamino-o-tolyl) methane  
 tris(p-hexylaminophenyl) methane  
 tris[p-bis(2-hydroxyethyl)aminophenyl] methane  
 tris(p-methylaminophenyl) methane  
 tris(p-diocadecylaminophenyl) methane  
 tris(4-diethylamino-2-fluorophenyl) methane  
 tris(4-dimethylamino-2-fluorophenyl) methane  
 bis(2-bromo-4-diethylaminophenyl) phenylmethane  
 bis(2-butoxy-4-diethylaminophenyl) phenylmethane  
 bis(4-diethylamino-o-tolyl) (p-methoxyphenyl) methane  
 bis(4-diethylamino-2-methoxyphenyl) (p-nitrophenyl)  
 methane  
 bis(4-diethylamino-1-naphthyl) (4-diethylamino-o-tolyl)  
 methane  
 bis(4-diethylamino-o-tolyl) 1-naphthylmethane  
 bis(4-diethylamino-o-tolyl) phenylmethane  
 tris(4-dimethylamino-2-chlorophenyl) methane  
 bis(4-dimethylamino-2,5-dimethylphenyl) phenylmethane  
 bis(4-dimethylamino-o-tolyl) (o-bromophenyl) methane  
 bis(4-ethylbenzylamino-o-tolyl) (p-methoxyphenyl)  
 55 methane  
 tris(p-diethylamino-o-tolyl) methane  
 bis(4-diethylamino-o-tolyl)-4-methoxy-1-naphthyl  
 methane  
 bis(4-diethylamino-o-tolyl)-3,4,5-trimethoxyphenyl  
 60 methane  
 bis(4-diethylamino-o-tolyl)-p-hydroxyphenyl methane  
 5-[bis(4-diethylamino-o-tolyl)-methyl]-2,3-cresotic acid  
 4-[bis(4-diethylamino-o-tolyl)-methyl]-phenol  
 4-[bis(4-diethylamino-o-tolyl)-methyl]-acetanilide  
 65 4-[bis(4-diethylamino-o-tolyl)-methyl]-phenylacetate  
 4-[bis(4-diethylamino-o-tolyl)-methyl]-benzoic acid  
 4-[bis(4-diethylamino-o-tolyl)-methyl]-diphenyl sulfone  
 4-[bis(4-diethylamino-o-tolyl)-methyl]-phenylmethyl  
 sulfone  
 70 4-[bis(4-diethylamino-o-tolyl)-methyl]-methylsulfon-  
 anilide  
 4-[bis(4-diethylamino-o-tolyl)-methyl]-p-tolylsulfon-  
 anilide  
 75 bis(4-diethylamino-o-tolyl)-p-nitrophenyl methane

bis(4-diethylamino-o-tolyl)(2-diethylamino-4-methyl-5-thiazolyl)methane  
 bis(4-diethylamino-o-tolyl)(2-diethylamino-5-methyl-6-benzoxazolyl)methane  
 bis(4-diethylamino-o-tolyl)(2-diethylamino-5-methyl-6-benzothiazolyl)methane  
 bis(4-diethylamino-o-tolyl)(1-ethyl-2-methyl-3-indolyl)methane  
 bis(4-diethylamino-o-tolyl)(1-benzyl-2-methyl-3-indolyl)methane  
 bis(4-diethylamino-o-tolyl)(1-ethyl-2-methyl-5-methoxyl-3-indolyl)methane  
 bis(1-o-xylyl-2-methyl-3-indolyl)(4-diethylamino-o-tolyl)methane  
 bis(4-diethylamino-o-tolyl)(1-ethyl-5-indolyl)methane  
 bis(1-isobutyl-6-methyl-5-indolyl)(4-diethylamino-o-tolyl)methane  
 bis(4-diethylamino-o-tolyl)(8-methyl-9-julolindinyl)methane  
 bis(4-diethylamino-2-acetamidophenyl)(4-diethylamino-o-tolyl)methane  
 4-[bis(4-diethylamino-o-tolyl)methyl]-N-ethylacetanilide  
 bis[4-(1-phenyl-2,3-dimethyl-5-pyrazolinyl)](4-diethylamino-o-tolyl)methane  
 bis(4-diethylamino-o-tolyl)(7-diethylamino-4-methyl-3-coumarinyl)methane  
 bis(4-diethylamino-o-tolyl)(4-acrylamidophenyl)methane  
 bis(4-diethylamino-o-tolyl)(p-benzylthiophenyl)methane  
 bis(4-diethylamino-o-tolyl)(4-isopropylthio-3-methylphenyl)methane  
 bis(4-diethylamino-o-tolyl)(4-chlorobenzylthiophenyl)methane  
 bis(4-diethylamino-o-tolyl)(2-furyl)methane  
 bis(4-diethylamino-o-tolyl)(3,4-methylenedioxyphenyl)methane  
 bis(4-diethylamino-o-tolyl)(3,4-dimethoxyphenyl)methane  
 bis(4-diethylamino-o-tolyl)(3-methyl-2-thienyl)methane  
 bis(4-diethylamino-o-tolyl)(2,4-dimethoxyphenyl)methane  
 bis[4-(2-cyanoethyl)(2-hydroxyethyl)amino-o-tolyl](p-benzylthiophenyl)methane  
 bis[4-(2-cyanoethyl)(2-hydroxyethyl)amino-o-tolyl]-2-thienylmethane  
 bis(4-dibutylamino-o-tolyl)2-thienylmethane  
 bis(4-diethylamino-2-ethylphenyl)(3,4-methylenedioxyphenyl)methane  
 bis(4-diethylamino-2-fluorophenyl)(p-benzylthiophenyl)methane  
 bis(4-diethylamino-2-fluorophenyl)(3,4-methylenedioxyphenyl)methane  
 bis(4-diethylamino-o-tolyl)(p-methylthiophenyl)methane  
 bis(4-diethylamino-o-tolyl)2-thienylmethane  
 bis(4-dimethylamino-2-hexylphenyl)(p-butylthiophenyl)methane  
 bis[4-(N-ethylanilino)-o-tolyl](3,4-dibutoxyphenyl)methane  
 bis[4-bis(2-hydroxyethyl)amino-2-fluorophenyl](p-benzylthiophenyl)methane  
 bis(4-diethylamino-o-tolyl)-p-chlorophenyl methane  
 bis(4-diethylamino-o-tolyl)-p-bromophenyl methane  
 bis(4-diethylamino-o-tolyl)-p-fluorophenyl methane  
 bis(4-diethylamino-o-tolyl)-p-tolyl methane  
 bis(4-diethylamino-o-tolyl)-4-methoxy-1-naphthyl methane  
 bis(4-diethylamino-o-tolyl)-3,4,5-trimethoxyphenyl methane  
 bis(4-diethylamino-o-tolyl)-p-hydroxyphenyl methane  
 bis(4-diethylamino-o-tolyl)-3-methylthienyl methane

The hexaarylbiiimidazoles are the 2,2',4,4',5,5'-hexaarylbiiimidazoles (sometimes referred to as 2,4,5-triarylimidazolyl dimers) that are dissociable to the corresponding triarylimidazolyl radicals wherein the aryl groups may be the same or different, carbocyclic or heterocyclic sub-

tituent free or bearing substituents that do not interfere with the dissociation step and the subsequent oxidation of the leuco aminotriarylmethane.

The hexaarylbiiimidazoles can be represented as the dimers of 2,4,5-triarylimidazolyls of the formula



10

20

25

30

40

45

50

55

60

70

wherein A, B, and D are aryl radicals, as previously defined.

The hexaarylbiiimidazoles can also be represented by the formula



wherein A, B and D stand for aryl radicals described above. In these dimers each imidazolyl ring has two conjugated double bonds and a single bond joining the two rings. Upon dissociation, the dimer forms the corresponding 2,4,5-triarylimidazolyl radical. The B and D groups can normally carry 0-3 substituents, the A group 0-4 substituents.

The aryl groups include one- and two-ring aryls, such as phenyl, biphenyl, naphthyl, pyridyl, furyl and thiienyl. Suitable inert substituents on the aryl groups have Hammett sigma (para) values in the -0.5 to 0.8 range and are other than hydroxyl, sulfhydryl, amino, alkylamino or dialkylamino. Preferably, these inert substituents are free of Zerewitinoff hydrogen, i.e., have no hydrogens reactive towards methyl magnesium iodide. Representative substituents and their sigma values (relative to H=0.00), as given by Jaffe, *Chem. Rev.* 53, 219-233 (1953) are: methyl (-0.17), ethyl (-0.15), t-butyl (-0.20), phenyl (0.01), butoxy (-0.32), phenoxy (-0.03), fluoro (0.06), chloro (0.23), bromo (0.23), iodo (0.28), methylthio (-0.05), nitro (0.78), ethoxycarbonyl (0.52), and cyano (0.63). The foregoing substituents are preferred; however, other substituents which may be employed include trifluoromethyl (0.55), chloromethyl (0.18), carboxyl (0.27), cyanomethyl (0.01), 2-carboxyethyl (-0.07), and methylsulfonyl (0.73). Thus, the substituents may be halogen, cyano, lower hydrocarbyl (including alkyl, halo alkyl, cyanoalkyl, hydroxyalkyl and aryl), lower alkoxy, aryloxy, lower alkylthio, arylthio, sulfo, alkyl sulfonyl, arylsulfonyl, and nitro, and lower alkylcarbonyl. In the foregoing list, alkyl groups referred to therein are preferably of 1-6 carbon atoms; while aryl groups referred to therein are preferably of 6-10 carbon atoms.

Preferably the aryl radicals are carbocyclic, particularly phenyl, and the substituents have Hammett sigma values in the range -0.4 to +0.4, particularly lower alkyl, lower alkoxy, chloro, fluoro, bromo and benzo groups.

In a preferred biimidazole class, the 2 and 2' aryl groups are phenyl rings bearing an ortho substituent having a Hammett sigma value in the range -0.4 to +0.4. Preferred ortho substituents are fluorine, chlorine, bromine, methyl and methoxy groups, especially chloro. Such dimers tend less than other dimers to form color when the light-sensitive compositions are applied to and dried on substrates at somewhat elevated temperatures, e.g. in the range 70-100° C.

Most preferably, the 2-phenyl ring carries only the above-described ortho group, and the 4- and 5-phenyl rings are either unsubstituted or substituted with lower alkoxy. The hexaarylbiimidazoles are conveniently prepared by oxidatively coupling the corresponding 2,4,5-triphenylimidazole, as disclosed in British Pat. 1,047,569. The preferred method involves oxidation with ferricyanide in alkali and generally yield the 1,2-biimidazoles, although other isomers such as the 1,1', 1,4', 2,2', 2,4', 4,4' biimidazoles are sometimes obtained. It is immaterial which isomer is employed in this invention so long as it is photodissociable.

Representative dimers of the imidazolyl radicals other than those given in the examples which fall within the scope of the invention are listed below, in terms of the substituents of the aryl groups when aryl is phenyl and in terms of other aryl groups than phenyl, by way of illustrating the activatable imidazolyl dimers which may be employed in the composition.

## I.—PHENYL SUBSTITUTED IMIDAZOLYL RADICALS

## SUBSTITUENTS OF PHENYL RINGS ATTACHED AT—

| 2-position                                   | 4-position               | 5-position              |   |
|----------------------------------------------|--------------------------|-------------------------|---|
| o-Acetoxy.....                               | .....                    | .....                   | 5 |
| o-Benzyl.....                                | o-Benzylthio.....        | o-Benzylthio.....       |   |
| o-Benzylthio.....                            | o-Benzylthio.....        | o-Benzylthio.....       |   |
| P-[4,5-bis(p-methoxy-phenyl)-2-imidazolyl].  | .....                    | o-Methoxy.....          |   |
| o-Bromo.....                                 | p-Bromo.....             | o-Methoxy.....          |   |
| Do.....                                      | o-Methoxy.....           | o-Methoxy.....          |   |
| 2-Bromo-4-phenyl.....                        | .....                    | .....                   |   |
| o-n-Butoxy.....                              | .....                    | .....                   |   |
| N-butyacetamido.....                         | .....                    | .....                   |   |
| o-Butylthio.....                             | .....                    | .....                   |   |
| p-t-Butylthio.....                           | .....                    | .....                   |   |
| o-Butyroxy.....                              | .....                    | .....                   |   |
| o-Chloro.....                                | o-Chloro.....            | o-Chloro.....           |   |
| Do.....                                      | p-Chloro.....            | o-Chloro.....           |   |
| Do.....                                      | do.....                  | p-Chloro.....           |   |
| Do.....                                      | 3,4-Dichloro.....        | .....                   |   |
| Do.....                                      | p-Methoxy.....           | .....                   |   |
| Do.....                                      | m-Pentyloxy.....         | .....                   |   |
| Do.....                                      | do.....                  | m-Pentyloxy.....        |   |
| Do.....                                      | m-Methoxy.....           | m-Methoxy.....          |   |
| 2-chloro-5-SO <sub>3</sub> H.....            | .....                    | .....                   |   |
| 2-chloro-4-phenyl.....                       | .....                    | .....                   |   |
| 2-chloro-4-methoxy.....                      | .....                    | .....                   |   |
| p-Chloro.....                                | p-Chloro.....            | p-Chloro.....           |   |
| o-Cyano.....                                 | p-t-Butyl.....           | p-t-Butyl.....          |   |
| Do.....                                      | do.....                  | .....                   |   |
| Do.....                                      | p-Cyano.....             | p-Cyano.....            |   |
| Do.....                                      | p-Methoxy.....           | p-Methoxy.....          |   |
| 2,3-dibromo.....                             | .....                    | .....                   |   |
| 2,4-dibromo.....                             | .....                    | .....                   |   |
| 2,6-dibutyl.....                             | .....                    | .....                   |   |
| o-Dibutylsulfamoyl.....                      | .....                    | .....                   |   |
| 2,4-dichloro.....                            | o-Bromo.....             | .....                   |   |
| 2,6-dichloro.....                            | Do.....                  | p-Butoxy.....           |   |
| 3,4-dichloro.....                            | 2,4-dimethoxy.....       | p-Butoxy.....           |   |
| 2,4-dicyano.....                             | p-Cyano.....             | p-Cyano.....            |   |
| 2,6-dicyano.....                             | .....                    | .....                   |   |
| 3,5-dicyano-4-methoxy.....                   | .....                    | .....                   |   |
| p-(2,2-dicyanovinyl).....                    | .....                    | .....                   |   |
| 2,4-diethoxy.....                            | .....                    | .....                   |   |
| o-Diethylsulfamoyl.....                      | .....                    | .....                   |   |
| 2,5-difluoro.....                            | p-Cyano.....             | .....                   |   |
| Do.....                                      | do.....                  | Do.....                 |   |
| 2,3-dimethoxy.....                           | o-Chloro.....            | o-Chloro.....           |   |
| 2,4-dimethoxy.....                           | Do.....                  | o-Chloro.....           |   |
| Do.....                                      | 2,4-dimethoxy.....       | 2,4-dimethoxy.....      |   |
| Do.....                                      | do.....                  | 2,4-dimethoxy.....      |   |
| Do.....                                      | o-Methoxy.....           | .....                   |   |
| Do.....                                      | do.....                  | p-Methoxy.....          |   |
| Do.....                                      | m-Phenylthio.....        | .....                   |   |
| Do.....                                      | do.....                  | m-Phenylthio.....       |   |
| 3,4-dimethoxy.....                           | o-Cyano.....             | 2,4-dipentyl.....       |   |
| Do.....                                      | 2,4-dipentyl.....        | 2,4-dipentyl.....       |   |
| 2,4-dimethoxy.....                           | o-Dimethylcarbamoyl..... | Do.....                 |   |
| 2,4-dipentyl.....                            | 2,4-dipentyl.....        | Do.....                 |   |
| p-(4,5-diphenyl-2-imidazolyl).....           | .....                    | .....                   |   |
| p-[4-(4,5-diphenyl-2-imidazolyl)phenyl]..... | .....                    | .....                   |   |
| 2,4-dipropoxy.....                           | .....                    | .....                   |   |
| 2,4-dinaphthylthio.....                      | m-Methoxy.....           | m-Methoxy.....          |   |
| 2-nitro.....                                 | .....                    | .....                   |   |
| 2-nitro-5-methoxy.....                       | .....                    | .....                   |   |
| 2,4-dipropoxy.....                           | o-Diethylcarbamoyl.....  | .....                   |   |
| o-Dipropylcarbamoyl.....                     | .....                    | .....                   |   |
| p-Ethoxy.....                                | Do.....                  | p-Diethylsulfamoyl..... |   |

## II.—OTHER RING GROUPS THAN PHENYL IN IMIDAZOLYL RADICAL

| 2-position                    | 4-position | 5-position  |
|-------------------------------|------------|-------------|
| 2,4-dipentylphenyl            | 2-naphthyl | 2-naphthyl  |
| p-Methoxyphenyl               | do         | Do.         |
| o-Methoxycarbonylphenyl       | do         | Phenyl.     |
| (1-methoxy-2-naphthyl)        | Phenyl     | Do.         |
| (3-methoxy-2-naphthyl)        | do         | Do.         |
| 1-naphthyl                    | do         | Do.         |
| o-Pentylmethoxycarbonylphenyl | 2-naphthyl | 2-naphthyl. |
| 3-pyridyl                     | Phenyl     | Phenyl.     |

The above dimers of 2,4,5-triarylimidazolyl radicals which provide light-activated components for the invention compositions are characterized by the property of dissociating into two triarylimidazolyl free radicals when illuminated with ultraviolet light of a wavelength from about 2000 Å. to 4200 Å. Such a dissociation may be detected, and the existence of the free radicals discerned, by electron paramagnetic resonance, by ultraviolet spectra, and by visible spectra.

## (3) OTHER COMPONENTS

Inert solvents are usually employed to dissolve the components of the composition of this invention and to provide a fluid medium for convenient application of the light-sensitive composition to substrates. To obtain the final coated article the solvent is normally removed as, e.g., by evaporation. It is often beneficial to leave a small residue of solvent in the dried composition so that the desired degree of imaging can be obtained upon subsequent irradiation. Ordinary drying such as that employed in paper manufacture or in film casting results in the retention of ample solvent to give a composition with good photosensitivity. The compositions so produced are dry to the touch and stable to storage at room temperature. Indeed, moisture of the air is absorbed by many of the compositions, particularly those comprising an acid salt of an amino leuco form of a dye on cellulosic substrates, and serves as a suitable solvent.

In general, suitable solvents have boiling points of at least 40° C. at atmospheric pressure, although solvents with higher boiling points may be used. Examples are amides such as N,N-dimethylformamide and N,N-dimethylacetamide; alcohols and ether alcohols such as methanol, ethanol, 1-propanol, 2-propanol, butanol, and ethylene glycol; esters such as methyl acetate and ethyl acetate; aromatics such as benzene, o-dichlorobenzene, toluene; ketones such as acetones, methyl ethyl ketone, 3-pentanone; aliphatic halo carbons such as methylene chloride, chloroform, 1,1,2-trichloroethane, 1,1,2,2-tetrachloroethane, 1,1,2-trichloroethylene; miscellaneous solvents such as dimethylsulfoxide, pyridine, tetrahydrofuran, dioxane, dicyanocyclobutane, 1-methyl-2-oxohexamethyleneimine; and mixtures of these solvents in various proportions may be required to attain solution of the color forming and color preventing compounds.

Polymeric binders may also be present in the light-sensitive compositions to thicken them or adhere them to substrates. Binders can also serve as a matrix for the color-forming composition and the mixture may be cast, extruded or otherwise formed into unsupported imageable films. Light-transparent and film-forming polymers, are preferred. Examples are ethyl cellulose, polyvinyl alcohol, polyvinyl chloride, polystyrene, polyvinyl acetate, poly(methyl methacrylate), cellulose acetate, cellulose propionate, cellulose butyrate, cellulose acetate butyrate, cellulose nitrate, chlorinated rubber, copolymers of the above vinyl monomers, and gelatin. Binder or matrix amounts vary from about 0.5 part to about 200 parts by weight per part of combined weight of the leuco triarylmethane and the hexaarylimidazole. In general from 0.5 to 10 parts are used as adhesive or thickener, while higher amounts are used to form the unsupported films. With certain polymers, it may be desirable to add

a plasticizer to give flexibility to the film or coating. As noted above the preferred classes of methyleneoxy hydrogen donors described above as reductants in the deactivation system also serve as plasticizers. Other plasticizers that may be used are the alkyl phthalates and phosphates, such as dimethyl phthalate, diethyl phthalate, dioctyl phthalate, tributyl phosphate, trihexyl phosphate, trioctyl phosphate, triphenyl phosphate, tricresyl phosphate and cresyl diphenyl phosphate.

## (4) PREPARATION OF THE COMPOSITIONS

A common procedure is to make a solution of a leuco triarylmethane defined as in (A) in the summary above ranging in concentration from about 0.5% by weight to 15 the limit of the solubility of the compounds in a solvent comprising, for instance, 50:50 by volume of N,N-dimethylformamide and benzene, and to add to this solution, in amounts set forth further above, the hexaarylimidazole defined as in (B), the quinones defined as in (C) and (D) and the ether reductant defined as in (E) and optionally a binder as described above. The selection of the leuco triarylmethane will depend upon the color and quality of the image desired. Two or more leuco triarylmethanes may be used in combination to obtain 25 a particular color or shade of color or to provide a neutral gray or black coloration in the image.

## (5) SUBSTRATES

In use, the compositions of this invention are usually 30 coated upon or impregnated in substrates. The substrates are materials commonly used in the graphic arts and in decorative applications and include paper ranging from tissue paper to heavy cardboard; films of plastics and 35 polymeric materials such as regenerated cellulose, cellulose acetate, cellulose nitrate, polyester of glycol and terephthalic acid, vinyl polymers and copolymers, polyethylene, polyvinylacetate, polymethyl methacrylate polyvinylchloride; textile fabrics; glass, wood and metals. 40 Opaque as well as transparent substrates can be used. Substrates in which the photosensitive components are dissolved or which bear the photosensitive components as a coating on the reverse side of the substrate, i.e., on the side away from the ultraviolet light source used for 45 image formation, must be transparent not only in the visible region but transparent to a portion of the ultraviolet range useful for image formation. The substrates must also be inert to the photosensitive materials and 50 preferably should not dissolve the active components but absorb them and retain sufficient solvent to provide a medium for rapid image formation upon irradiation.

In applying a solution to paper, films, fabrics, or to 55 the surface of rigid substrates such as glass, wood or metals the solution may be sprayed, brushed, applied by a roller or an immersion coater, flowed over the surface, picked up by immersion or spread by other means. Complete coverage of the substrate may be attained or 60 a pattern of the light-sensitive composition may be printed on the substrate. In impregnating paper, for instance, such concentrations of solution and pick-up by the paper are made so as to provide from about 0.01 mg./in.<sup>2</sup> to about 5.0 mg./in.<sup>2</sup> of the triarylmethane and equivalent amount of the hexaarylimidazole. Images of greater 65 and lesser intensity of color are provided by the application of greater and lesser amounts of the triarylmethane to the substrate. For coating roll papers and films there may be used such typical devices for continuously laying down wet films as nip fed three roll reverse roll coating heads, gravure coaters, trailing blade coaters and Mayer bar coating heads (wherein the coating thickness is controlled by a threaded or a wire wound bar). The wet thickness is adjusted such that the dry thickness after solvent removal is in the desired range (about 0.1-1.5 mils, usually around 0.3-0.5 mil on paper, 0.8-1.1 mils on film).

The substrates bearing a solution of the compositions of this invention may be dried simply at room temperature. They also may be dried under vacuum at room temperature by forced air solvent evaporation, or at elevated temperatures, as by radiant heating. The upper temperature limit is important in combination with exposure time. A short exposure to heat of 90° C. may not be detectably harmful, while several hours exposure to this heat may reduce the light sensitivity of the composition.

#### (6) LIGHT SOURCES, IMAGE FORMATION AND DEACTIVATION

Any convenient source of ultraviolet light may be used to activate the color-forming system to induce the formation of an image, whereas convenient sources of visible light may be used to achieve deactivation. In general, light sources that supply radiation in the region between about 2000 Å. and about 4200 Å. are useful in producing images with the leuco triarylmethane/hexaaryl-biimidazole compositions on numerous substrates. Light sources generating radiation in the region between about 4200 Å. and about 5500 Å. are useful to achieve deactivation. Among the light sources which have been employed are sunlamps, pulsed and continuous Xenon flash lamps, germicidal lamps, ultraviolet lamps providing specifically light of short wavelength (2537 Å.) and lamps providing light of longer wavelengths, narrow or broad band, centered near 3600 Å., 4200 Å., 4500 Å., or 5000 Å., such as fluorescent lamps, mercury, metal additive and arc lamps. The light exposure time will vary from a fraction of a second to several minutes, depending upon the intensity and spectral energy distribution of the light, its distance from the composition, the nature and amount of the composition available, and the intensity of color in the image desired. There may also be used coherent light beams, for example, pulsed nitrogen lasers, argonion lasers and ionized neon lasers, whose emissions fall within or overlap the ultraviolet absorption bands of the hexaarylbiimidazole or visible absorption bands of the quinones.

Ultraviolet or visible emitting cathode ray tubes widely useful in printout systems for writing on photosensitive materials are also useful for imaging the subject compositions. These in general involve a UV- or visible-emitting phosphor internal coating as the means for converting electrical energy to light energy and a fiber optic face plate as the means for directing the radiation to the photosensitive target. For purposes of this invention, the phosphors should emit strongly below 420 m $\mu$  (4200 Å.) so as to substantially overlap the near UV-absorption characteristic or between about 420 m $\mu$  to about 550 m $\mu$  to overlap the visible absorption characteristics of the novel imaging compositions. Representative phosphors include the P4B (emitting at 300-550 m $\mu$ , peaking at 410 m $\mu$ ), P16 (330-460 m $\mu$ , peaking at 380 m $\mu$ ) and P22B (390-510 m $\mu$ , peaking at 450 m $\mu$ ) types. Other phosphors which may be used are the P11 (400-560 m $\mu$ , peaking at 460 m $\mu$ ) and ZrP<sub>2</sub>O<sub>7</sub> types. (The Electronic Industries Association, New York, N.Y., assigns P-numbers and provides characterizing information on the phosphors; phosphors with the same P-number have substantially identical characteristics.)

Of course, it is to be understood that sources emitting principally in the ultraviolet will be most effective for activation. In instances where a light source emits strongly in both regions, optical filters will be required to both eliminate the visible components for effective color formation and to permit deactivation without undesired color formation.

Images may be formed by a beam of light or by exposure to light of a selected area behind a negative, a stencil, or other relatively opaque pattern. The negative may be a silver negative with cellulose acetate or polyester film. The negative may also be one in which the

opacity results from aggregations of areas of different refractive index. Image formation may also be accomplished in conventional diazo printing apparatus, or in a thermography device, provided the instrument emits some of its light in the ultraviolet range. A piece of onion-skin paper which bears typewriting, for example, will serve as a master pattern from which copies can be made.

The subject compositions are also activatable for the purposes of this invention by electron beams. The optimum conditions depend on the formulation and its thickness, the electron beam energy and the exposure time, and are readily determined by trial. Beams having average electron energies as low as about 10 kilovolts and as high as about 2 million electron volts have been used successfully.

The deactivating radiation employed is visible light radiation. A notable feature of this invention is that no other deactivating conditions are necessary. Thus no special precautions need be taken to prevent concurrent imaging under ambient light conditions. Negative images stable to ambient light are obtained by imagewise exposing the composition to ultraviolet light. Positive images are obtained by first imagewise exposing the composition to visible light until the desired degree of deactivation in the exposed area is attained, followed by developing the resulting latent image by exposing the composition to ultraviolet light.

#### (7) USEFULNESS

The novel compositions of this invention are useful in such diverse fields as optical printing and image-recording, generally, dyeing of textiles and other materials, photography, thermography and pattern layout. The compositions are also useful to sense thresholds of light, heat, pressure and combinations thereof, through the color changes they undergo when activated by such stimuli. Some specific uses are:

(1) Radiation dosimeters.—These compositions may be used as papers to determine easily the quantity of solar radiation that falls on a particular surface. It may also be useful to employ these as low cost light-meters in photographic applications. For these uses, it is necessary to compare areas which have been exposed to previously calibrated papers or surfaces, in order to allow easy analysis of the degree of radiation.

(2) Blue prints.—These light-sensitive compositions can find application in diazo printout equipment, where they can be made to give readily a variety of shades, with different speeds and sensitivities. It is possible to utilize these materials with caution in ordinary room light, rather than have to handle them in the dark.

(3) Printing applications.—This invention is particularly useful for light-actuated colored image formation and provides a dry, non-silver photographic process capable of imaging in various colors and shades on various substrates, including fabrics, paper and similar fibrous sheet material. Apparatus useful in conducting photographic dye-printing is described in U.S. Pats. 2,214,365 and 2,655,802. Even very soft paper, as for example tissue paper, which has been treated with a composition of this invention can be readily printed by projecting the desired graphic pattern onto the treated paper and irradiating it to effect the color-forming oxidation reaction. Subsequently, the image is fixed as described heretofore. These soft tissue paper compositions cannot be readily imaged by conventional printing techniques.

In general the compositions of this invention are broadly useful for optical printing and anywhere it is desirable to capture images as in photography, pattern-making, reproducing written, printed, drawn or typed matter, and recording radiation signals as line graphics, alpha-numerics or other characters. The applied radiation can be passed through stencils, negatives or transparencies including halftone and continuous tone nega-

tives and positives in contact with or projected onto the composition; or, it can be reflected for impingement on the composition from printed or typed copy or objects that are opaque or transmit radiation poorly. Similarly, images of objects having areas differing in absorption and transmission characteristics are captured by placing the objects between the color forming radiation source and the composition, e.g., foot images can be recorded for fitting shoes. Multiple copies can be made using a single imaging exposure by stacking radiation-transparent assemblies comprising the composition coated on a transparent substrate such as UV-transparent film, paper or glass.

In imaging applications, the ultimately desired dye optical density pattern can be constructed stepwise, according to one or more patterns, by exposing previously unexposed areas to suitable activating radiation and/or by reexposing previously under exposed areas (i.e., areas wherein the maximum obtainable optical density has not yet been fully developed) to one or more additional exposures. Such "add on" capability and versatility of the invention compositions is particularly useful in recording information and creating electronically generated displays and graphics. Because the recorded images have excellent resolution on paper and film, they are suitable for micro-imaging for data storage. Information stored on such microfilms can be printed out on other microfilms, if desired.

The following examples illustrate the invention in greater detail.

#### Example 1

A coating composition was prepared by mixing the following:

| Ingredients                                                                                      | Parts  | Molar proportions |
|--------------------------------------------------------------------------------------------------|--------|-------------------|
| Acetone.....                                                                                     | 46.0   |                   |
| Cellulose acetate butyrate.....                                                                  | 6.0    |                   |
| p-Nonylphenol-ethylene oxide adduct, $C_9H_{19}C_6H_4O$<br>( $CH_2CH_2O$ ) <sub>1.8</sub> H..... | 4.0    | 1.92              |
| Tris(p-diethylaminoethyl-o-tolyl)methane.....                                                    | 0.300  | 0.75              |
| p-Toluenesulfonic acid monohydrate.....                                                          | 0.344  | 2.25              |
| 2-(o-chlorophenyl)-4,5-(m-methoxyphenyl)-imidazolyl dimer.....                                   | 0.624  | 1.00              |
| 1,6- and 1,8-pyrenequinones, added as a 1:1 mixture.....                                         | 0.0371 | 0.2               |
| 9,10-phenanthrenequinone.....                                                                    | 0.0664 | 0.4               |

<sup>1</sup> 92 methyleneoxy groups/mole quinone mixture.

The solution was applied to bleached-sulfite roll stock paper and the acetone allowed to evaporate to give a coating about 0.4 mil thick. The coated composition rapidly developed a deep blue color when exposed to ultraviolet light, for example, on contact flashing with a Xenon flash lamp (HiCo Lite, emitting UV and visible light and approximating unfiltered sunlight) through a Corning 7-54 filter which cuts off wavelengths above 420 mu.

This composition can be completely deactivated against UV-induced color formation by irradiation with 4360 A. light using a Bausch and Lomb monochromator and an Osram HBO 200-watt mercury lamp at an intensity of 15-milliwatts per square centimeter of exposed surface for 70 seconds.

The marked deactivation capability of this formulation under various ambient lighting conditions, that is, its resistance to develop unwanted color under room light, daylight and sunlight conditions is illustrated with the following stability tests:

Roomlight—24 hour exposure to light from a cool white fluorescent lamp at 50 foot candles.

Daylight—10 minute exposure to sky illumination at midmorning in winter with the photosensitive surface perpendicular to the ground and facing southwest at a location of about 34° north and about 77° west at about sea level.

Sunlight—1 minute exposure to direct sunlight at mid-afternoon in winter with the photosensitive surface per-

pendicular to the ground and facing southwest at the same location as for the daylight test.

The results are tabulated below along with results obtained with formulations representative of the prior art. For these comparisons, coated papers were prepared as described above except that mixed quinones employed in the formulation set forth above were replaced by the quinones as set forth immediately below:

|    | Quinone, millimoles | Increase in optical density over background and color |              |           |          |          |
|----|---------------------|-------------------------------------------------------|--------------|-----------|----------|----------|
|    |                     | Pyrene                                                | Phenanthrene | Roomlight | Sunlight | Daylight |
|    |                     |                                                       |              |           |          |          |
| 15 | Example 1.....      | 0.16                                                  | 0.32         | 1 0.23    | 1 0.01   | 1 0.16   |
|    | Comparative:        |                                                       |              |           |          |          |
|    | A.....              | 0.16                                                  |              |           | 2 0.53   | 2 0.91   |
|    | B.....              | 0.32                                                  |              | 3 0.28    | 2 0.58   | 2 0.78   |
|    | C.....              |                                                       | 0.32         |           | 2 0.48   | 2 0.65   |
|    | D.....              |                                                       | 0.48         |           | 1 0.15   | 2 0.41   |

<sup>1</sup> Buff. <sup>2</sup> Blue. <sup>3</sup> Yellow buff.

#### The data show

(1) The invention composition is sufficiently stable to ambient light conditions so as not to require irradiation under controlled conditions for deactivation (image fixing).

(2) Neither the pyrenequinones alone nor the phenanthrenequinone alone provide for satisfactory daylight and sunlight stability particularly against the relatively long direct daylight exposure with its relatively high proportion of UV radiation.

(3) The mixed quinones of the invention provide for an aesthetically more appealing background color (buff versus yellow buff).

It should be noted that it is not practical to improve the stability of the prior art type formulation by increasing the proportion of either the pyrenequinone or the phenanthrenequinone since (a) large amounts of the pyrenequinones cause precipitation in storage, and (b) larger amounts of the phenanthrenequinones tend to decrease the imaging speed and the color developing capability of the system.

#### Example 2

A photodeactivatable photoimaging composition is prepared as in Example 1 except that the quinone mixture contains.

(a) 0.08 millimole of an approx. 1:1 mixture of 1,6- and 1,8-pyrenequinone and  
(b) 0.08 millimole of 9,10-phenanthrenequinone.

This composition is identical to a control composition in its color forming speed and in the amount of color developed on exposure to ultraviolet light (the control being essentially the same composition except that it contains .16 millimole of the pyrenequinones and no phenanthrenequinone). Like the control, this example composition is deactivated completely when exposed to 4360 A. light at 15 mw./cm.<sup>2</sup> intensity for 70 seconds. It is significantly more stable than the control in storage, showing a substantially lesser tendency to form precipitates. Moreover it is significantly more stable against color formation by direct daylight and sunlight exposure, giving lighter and less colored background than the control.

#### Examples 3 and 4

Example 1 was repeated with pyrenequinone (as the 1,6- and 1,8- approx. equimolar mixture) in combination with another quinone that can be employed in the compositions of this invention as identified below replacing the 9,10-phenanthrenequinone. The results are tabulated below in terms of the daylight and sunlight stability of the coated compositions; and are compared with compositions employing quinones in place of 9,10-phenan-

threnequinone that do not fall within the scope of this invention:

| Quinone (.32 millimoles)        | Increase in optical density<br>after exposure to— |          |
|---------------------------------|---------------------------------------------------|----------|
|                                 | Daylight                                          | Sunlight |
| Example:                        |                                                   |          |
| 3. Perinaphthenone              | 0.56                                              | 0.08     |
| 4. 4-methoxy-1,2-naphthoquinone | 0.41                                              | 0.05     |
| Comparative:                    |                                                   |          |
| E. 1-methoxyanthraquinone       | 0.70                                              | 0.33     |
| F. Phenazine                    | 0.70                                              | 0.30     |

The compositions of Examples 3 and 4 are remarkably stable to sunlight (relatively rich in visible light) though they are less stable to prolonged direct daylight exposure (relatively rich in ultraviolet) than is the Example 1 composition also containing 9,10-phenanthrenequinone as a photooxidant component.

#### Example 5

A coated substrate was prepared essentially as described in Example 1 except that the quantity of acetone was increased to 61 parts in the coating formulation and the composition was coated on "Mylar" polyester film to give a coating 0.7 to 0.8 mil thick.

The coated film showed good imaging (blue color forming) characteristics on exposure to ultraviolet light. It developed an optical density of only 0.18 (buff color) in the daylight stability test compared to 0.61 (blue) for the same coated film containing the pyrenequinones but no phenanthrenequinone.

#### Example 6

Substantially similar results are obtained on increasing the 2-(o-chlorophenyl)-4,5-(m-methoxyphenyl)imidazolyl dimer concentration from 0.8 to 1.6 millimoles in the above invention composition of Example 5.

#### Examples 7-18

Photodeactivatable photoimaging compositions having improved roomlight, daylight and sunlight stability against unwanted color formation are prepared as in Example 1 except that the p-nonylphenol/ethylene oxide adduct used as the reductant for the quinone mixture is replaced by an equal weight of an abstractable-hydrogen source containing one or more



groups as identified below where R=H or CH<sub>3</sub>:

| Reductant for pyrenequinone and phenanthrenequinone          | Number of<br>R<br>—CH—O—<br>groups per<br>mole Q | Example:                                                 |                                               |
|--------------------------------------------------------------|--------------------------------------------------|----------------------------------------------------------|-----------------------------------------------|
|                                                              |                                                  | 7. p-Phenylphenol/5.9 ethylene oxide adduct <sup>1</sup> | 8. o-Phenylphenol/2.25 ethylene oxide adduct. |
| 9. p-Cresol/1.5 ethylene oxide adduct                        | 144                                              | 230                                                      | 134                                           |
| 10. p-Cresol/2.25 ethylene oxide adduct                      | 180                                              |                                                          |                                               |
| 11. p-Cresol/3.0 ethylene oxide adduct                       | 208                                              |                                                          |                                               |
| 12. p-Cresol/2.0, 1,2-propylene oxide adduct                 | 150                                              |                                                          |                                               |
| 13. p-Cresol/1.25 ethylene oxide/2.0 propylene oxide adduct  | 194                                              |                                                          |                                               |
| 14. p-Cresol/3 ethylene oxide adduct acetate <sup>2</sup>    | 176                                              |                                                          |                                               |
| 15. p-Cresol/3 ethylene oxide adduct propionate <sup>2</sup> | 168                                              |                                                          |                                               |
| 16. Triethylene glycol dipropionate                          | 192                                              |                                                          |                                               |
| 17. 2-[2-butoxyethoxy]ethyl acetate                          | 204                                              |                                                          |                                               |
| 18. Dipropionin (glycerol dipropionate)                      | 122                                              |                                                          |                                               |

<sup>1</sup> Adduct signifies the alkylene ether product of the reaction of the phenol with 5.9 (or otherwise indicated) molar proportions of ethylene oxide.

<sup>2</sup> The terminal hydroxy group of the adduct has been esterified with the indicated acyl group.

#### Example 19

Coated paper was prepared as in Example 1 except that the coating formulation contained the following leuco dyes in place of the tris(p-diethylamino-o-tolyl) methane of Example 1: 0.3323 part of bis(p-diethylamino-o-tolyl) (3,4-dimethoxyphenyl)methane and 0.0898 part of bis(p-diethylamino-o-tolyl) (p-chlorophenyl) methane.

This formulation on exposure to ultraviolet light afforded pleasing gray to black images. Like the invention formulation of Example 1, it showed good roomlight, daylight and sunlight stability. Also it was markedly superior in its photodeactivation capability to the comparable formulation containing either the pyrenequinone or the phenanthrenequinone component.

#### Example 20

A coated paper prepared as in Example 1 was tested for resistance to fingerprinting against another coated paper representative of the photosensitive materials described in U.S. Pat. 3,390,994. The coating composition of said patent contained acetone (46 parts), cellulose acetate butyrate (6 parts), the nonylphenol/ethyleneoxide adduct of Example 1 (3 parts), the biimidazole (.209 part) and leuco dye (.045 part) of Example 1, p-toluenesulfonic acid monohydrate (.200 part), pyrenequinone (1:1 mixture of 1,6- and 1,8-isomers, .0302 part), and trimethyl nitrilotripropionate (.600 part) as the primary reductant for the quinone.

The fingerprinting test was conducted by touching the coated surface of each paper with a finger tip. The paper was then placed in an envelope, which was sealed, and stored in the dark. After 24 hours the paper was removed from the envelope and exposed to ultraviolet radiation for color development.

The paper coated with the composition of this invention showed uniform color development over the entire light struck area with no sign of a fingerprint. In contrast, the control composition clearly showed in the light struck area a substantially uncolored fingerprint where the coating had originally been touched.

Remarkably similar fingerprinting results are obtained when the paper substrate is finger-touched before the photosensitive coating is applied and the procedure is repeated.

Substantially the same fingerprinting results are obtained when a mixture of phenanthrenequinone and the pyrenequinones are employed in the above control formulation, indicating that the absence of the nitrilotripropionate component is necessary to achieve the resistance to fingerprinting which characterizes the compositions of this invention.

#### Example 21

An ambient light-stable photosensitive imaging composition of this invention was prepared to contain:

| 60 | Ingredients                                     | Parts  | Molar proportions |
|----|-------------------------------------------------|--------|-------------------|
|    | Acetone                                         | 46     |                   |
|    | Cellulose acetate                               | 6      |                   |
|    | Polyethylene glycol, mol. wt. 550               | 4      | 1.500             |
|    | Tris(p-diethylaminoethyl-o-tolyl)methane        | 0.30   | 0.75              |
| 65 | p-Toluenesulfonic acid, monohydrate             | 0.34   | 2.25              |
|    | 2-(o-chlorophenyl)-4,5-diphenylimidazolyl dimer | 0.53   | 1.00              |
|    | 1,6-pyrenequinone                               | 0.0047 | 0.025             |
|    | 1,8-pyrenequinone                               | 0.0047 | 0.025             |
|    | 9,10-phenanthrenequinone                        | 0.067  | 0.4               |

<sup>1</sup> 500 methyleneoxy groups per mole of combined quinones.

This composition showed good imaging speed and depth of color development upon irradiation with ultraviolet light. It is readily deactivated to a near white background on irradiation under standard conditions with 4360 Å. light at 15 mw./cm.<sup>2</sup> for 70 seconds, and is substantially

stable to cool white fluorescent light at a distance of 4 inches for one hour. In contrast, omitting either the pyrenequinones or the phenanthrenequinone from the above formulation results in compositions which are substantially less stable to room light; that is, they form some blue color under the above conditions.

The preceding representative examples may be varied within the scope of the present total specification disclosure, as understood and practiced by one skilled in the art, to achieve essentially the same results.

The foregoing detailed description has been given for clearness of understanding only and no unnecessary limitations are to be understood therefrom. The invention is not limited to the exact details shown and described, for obvious modifications will occur to those skilled in the art.

The embodiments of the invention in which an exclusive property or privilege is claimed are defined as follows:

**1. A photosensitive composition comprising an intimate admixture of**

- (A) a salt of a leuco triarylmethane and an acid;
- (B) a hexaarylbimidazole which absorbs principally in the ultraviolet region and is a photooxidant for the salt of the leuco triarylmethane present in an amount of from about 1 to 2 moles per mole of said salt of the leuco triarylmethane;
- (C) 1,6-pyrenequinone or 1,8-pyrenequinone or both, present in an amount of from about 0.04 to 0.4 mole per mole of hexaarylbimidazole;
- (D) a visible light-absorbing carbonyl compound selected from 9,10-phenanthrenequinone, perinaphthenone, or 4-methoxy-1,2-naphthoquinone; present in an amount of from about 0.05 to 2 moles per mole of hexaarylbimidazole; and
- (E) an ether containing at least one oxymethylene group wherein the methylene bears at least one hydrogen; present in an amount providing from about 50 to 500 oxymethylene groups per mole of the combined quinone components (C) and (D).

**2. The composition of claim 1 wherein**

in the leuco triarylmethane at least two of the aryl groups are phenyl groups having (a) an  $R_1R_2N$ -substituent in the position para to the bond to the methane carbon atom wherein  $R_1$  and  $R_2$  are each groups selected from hydrogen,  $C_1$  to  $C_{10}$  alkyl, 2-hydroxyethyl, 2-cyanoethyl, benzyl or phenyl, and (b) a group ortho to the bond to the methane carbon atom which is selected from lower alkyl, lower alkoxy, fluorine, chlorine, bromine, or butadienylene which when joined to the phenyl group forms a naphthalene ring; and the third aryl group, when different from the first two, is selected from thienyl, furyl, oxazolyl, pyridyl, thiazolyl, indolyl, indolinyl, benzoxazolyl, quinolyl, benzothiazolyl, phenyl, naphthyl, or such aforelisted groups substituted with lower alkyl, lower alkoxy, methylenedioxy, fluoro, chloro, bromo, amino, lower alkylamino, lower dialkylamino, lower alkylthio, hydroxy, carboxy, carbonamido, lower carbalkoxy, lower alkylsulfonyl, lower alkylsulfonamido,  $C_6$  to  $C_{10}$  arylsulfonamido, nitro or benzylthio,

the hexaarylbimidazole is a 2,2',4,4',5,5'-hexaphenyl-bimidazole in which the phenyl groups can contain substituents having Hammette sigma values of from -4 to +4.

**3. The composition of claim 1 wherein**  
the leuco triarylmethane has the structural formula



wherein  $R_3$  and  $R_4$  are selected from lower alkyl or

benzyl;  $Y$  and  $Y'$  are lower alkyl; and  $X$  is selected from



p-methoxyphenyl, 2-thienyl, phenyl, 1-naphthyl, 2,3-dimethoxyphenyl, 3,4-methylenedioxyphenyl, or p-benzylthiophenyl;

the hexaarylbimidazole is a 2,2',4,4',5,5'-hexaphenyl-bimidazole in which the 2 and 2' phenyl rings each bear an ortho substituent selected from fluorine, chlorine, bromine, methyl or methoxy; and the 4, 4', 5 and 5' phenyl groups each are either unsubstituted or bear a lower alkoxy substituent;

the pyrenequinone present is an approximately equimolar mixture of 1,6-pyrenequinone and 1,8-pyrenequinone;

the visible light-absorbing carbonyl compound is phenanthrenequinone; and  
the ether has the structural formula



wherein  $n$  is an integer of 0 or 1;  $m$  is an integer of 1 to 15;  $R$  is selected from hydrogen, alkyl, phenyl, alkphenyl, biphenyl or acyl wherein alkyl, alk- and acyl each contain 1 to 18 carbon atoms; and  $R'$  is hydrogen when  $n$  is 0, and is hydrogen, hydroxy or OR when  $n$  is 1.

**4. The composition of claim 3 wherein the ether has the formula**



wherein  $m$  is an integer of 1-15;  $R$  is phenyl, alkylphenyl of 7-25 carbon atoms, or biphenyl.

**5. The composition of claim 3 wherein**  
the hexaarylbimidazole is present in an amount of from about 1 to 2 moles per mole of the salt of the leuco triarylmethane;

the pyrenequinone mixture is present in an amount of from about 0.1 to 0.3 mole per mole of hexaarylbimidazole;

the 9,10-phenanthrenequinone is present in an amount of from about 0.15 to 0.75 mole per mole of hexaarylbimidazole, and

the ether is present in an amount providing from about 50 to 500 oxymethylene groups per mole of the quinones present.

**6. The composition of claim 1 wherein**  
the leuco triarylmethane is tris(p-diethylaminoethyl-o-tolyl)methane;

the hexaarylbimidazole is 2,2-bis(o-chlorophenyl)-4,4',5,5'-tetra(m-methoxyphenyl)biimidazole;

the pyrenequinone is an approximately equimolar mixture of 1,6-pyrenequinone and 1,8-pyrenequinone; the visible light-absorbing carbonyl compound is 9,10-phenanthrenequinone; and  
the ether is an adduct of p-nonylphenol and ethylene oxide.

**7. The composition of claim 1 wherein**  
the leuco triarylmethane is a mixture of bis(p-diethylamino-o-tolyl) (3,4-dimethoxyphenyl) methane and bis(p-diethylamino-o-tolyl) (p-chlorophenyl) methane;

the hexaarylbimidazole is 2,2-bis(o-chlorophenyl)-4,4',5,5'-tetra(m-methoxyphenyl)biimidazole;

the pyrenequinone is an approximately equimolar mixture of 1,6-pyrenequinone and 1,8-pyrenequinone; the visible light-absorbing carbonyl compound is 9,10-phenanthrenequinone; and  
the ether is an adduct of p-nonylphenol and ethylene oxide.

**21**

- 8. The composition of claim 1 coated on a substrate.
- 9. The composition of claim 1 coated on paper.
- 10. The composition of claim 1 coated on a synthetic film.
- 11. The composition of claim 1 impregnated in a substrate.
- 12. The composition of claim 1 combined with a plasticizer binder matrix.
- 13. The composition of claim 12 in the form of a self-supporting film.

**22**

- 14. The composition of claim 1 in admixture with an inert solvent.

**References Cited****UNITED STATES PATENTS**

- 5 3,390,994 7/1968 Cescon.
- 3,390,996 7/1968 McLachlan.

NORMAN G. TORCHIN, Primary Examiner

10 R. E. FICHTER, Assistant Examiner